

July 20, 1937.

J. W. STARK

2,087,389

WOVEN FABRIC

Filed Oct. 12, 1935

*Fig. 1*



*Fig. 2*



*Fig. 3*



*Fig. 4*



INVENTOR

*Joseph W. Stark*

BY

*Watson, Bristol, Johnson & Leavenworth*

ATTORNEYS

## UNITED STATES PATENT OFFICE

2,087,389

## WOVEN FABRIC

Joseph W. Stark, New York, N. Y., assignor to  
General Ribbon Mills, Incorporated, Catasau-  
qua, Pa., a corporation of Pennsylvania

Application October 12, 1935, Serial No. 44,657

11 Claims. (Cl. 139—420)

This invention relates in general to lustrous fabrics for decorative purposes and in particular to a non-reversible fabric, and to correlated improvements designed to enhance the lustre and decorative appearance of the same.

5 It is a general object of the invention to provide a fabric characterized by having a high lustre and a plurality of color effects.

10 It is a specific object of the invention to provide a fabric comprising strips of material having a metallic lustre, the lustrous material being associated with other materials capable of strengthening and enhancing the decorative effects of the lustrous strips.

15 A further object of the invention is the provision of fabric comprising strands each including a layer of transparent material laminated to a backing material with an adhesive which imparts to the fabric a desired color effect.

20 Other objects of the invention will in part be obvious and will in part appear hereinafter.

25 In accordance with the present invention, a lustrous fabric for decorative purposes is prepared by the use of strands comprising a plurality of flat strips cut from a laminated sheet material comprising at least two layers or sheets of flexible material laminated with a colored opaque adhesive, at least one of said layers or sheets being sufficiently transparent to reveal the color of the adhesive and at least one of the 30 layers being opaque and having a highly reflective surface.

35 For the weft of the fabric, there may be employed threads formed of textile fibres such, for example, as rayon, silk, wool, cotton, or flat threads formed of a transparent material such, for example, as viscose artificial horsehair filaments having a substantially flat cross-section and/or flat bands cut from a sheet of transparent, flexible sheet material such, for example, as regenerated cellulose, cellulose derivatives, gelatin, casein and other non-fibrous materials.

40 The invention accordingly comprises a new and improved article having the elements and the relation of elements, one to another, all as set forth in the following detailed description and the scope of the application of which will be indicated in the claims.

45 For a more complete understanding of the nature and objects of the invention, reference should be had to the accompanying drawing, in which:

50 Fig. 1 is a sectional view of one embodiment of one of the strands used in the improved fabric of the invention;

55 Fig. 2 is a sectional view of a second embodiment of one of the strands used in the invention;

Fig. 3 is a sectional view of another embodiment of a strand used in the invention; and

60 Fig. 4 is a perspective view with parts broken

away of one embodiment of the fabric of the invention.

For the transparent layer used in the warp strand, there may be employed any suitable flexible, non-fibrous sheet material such, for example, as regenerated cellulose, cellulose derivatives, gelatin, casein, polymerized vinyl resin or other synthetic resin, chlorinated rubber, as well as fibrous sheet materials which have been rendered substantially transparent by processing such, for example, as oiled silk, glassine paper and the like. The second layer of sheet material with which the transparent layer is laminated is preferably opaque and may comprise any suitable flexible sheet material such, for example, as paper, textile fabric, leather, metal foil or a sheet material having a metallic lustre formed by coating, spraying or laminating the sheet material with metal.

The adhesive used for laminating the sheet materials in forming the flat warp strand of the 20 fabric may comprise any suitable colored adhesive material which has been colored, for example by the addition of a coloring matter such as a dyestuff or a pigment, and the coloring matter may be transparent or opaque. Where one or 25 more of the laminae consists of sheet materials which may be wetted by water, the adhesive may be a water-soluble adhesive or formed of a water-swelling adhesive material such, for example, as glue, gelatin, agar, dextrine, starch, gum tragacanth and the like, or mixtures of the same made into a paste with water. If both of the laminae consist of sheet materials, the surfaces of which are not wetted by water, the adhesive may consist of an organic water-insoluble material such, for 30 example, as gums, resins, rubber or mixtures of the same dissolved in a suitable organic solvent.

35 Referring to the drawing, there is shown in Fig. 1 a simple embodiment of a suitable warp strand for use in the fabric of the invention. 40 This strand comprises a layer 10 of transparent material united by a layer 11 of colored adhesive to a layer 12 of opaque material. If desired, as shown in Fig. 2, the layer 10 of transparent material may be coated on both sides with a coating 45 13 of a transparent moistureproof composition adapted to protect the layer 10 from variations in humidity of the ambient atmosphere. In the embodiment of the warp strand shown in Fig. 3 the layer 12 of opaque material is coated on its 50 outer surface with a layer 14 of metal, either in the form of a lacquer containing metal particles or a layer of metal foil.

A preferred embodiment of the fabric of the invention is shown in Fig. 4, of which the warp 55 is formed of flat strands 15, each comprising a layer 10 of transparent material, such as regenerated cellulose, laminated with a layer 11 of a colored adhesive to a layer 12 of metal foil. In this embodiment the filler or weft comprises 60

threads 16 of rayon or the like woven through the warp strands 15 at spaced intervals so as not to detract substantially from the appearance of the warp strands. The fabric thus formed, as shown in Fig. 4, is a non-reversible material, the properties of the upper surface 17 being determined by the layer 10 of lustrous, transparent material and by the color and opacity of the layer 11 of adhesive, while the properties of the reverse surface 18 are determined by the nature of the backing material 12 which, in the fabric shown, consists of metal foil which imparts to this surface a high metallic luster.

The invention also contemplates employing two or more warp strands in which the layer 11 of adhesive varies in color or shade of color, whereby new and novel color effects are produced. For example, a group composed of a given number of warp strands may each comprise a laminated material as shown in Fig. 1 in which the adhesive has been colored dark green, while adjacent to this group there may be disposed a second group of warp strands in which the adhesive is colored a lighter shade of green. Accordingly, the present invention provides a new and novel method of obtaining a wide variety of colors in the warp strands simply by varying the color or the shade of color of the adhesive used in laminating the sheet materials comprising these strands. This obviates the expense entailed by employing strands cut from sheet materials which are themselves colored different colors or different shades of the same color.

It is another feature of the fabric that the layer 10 of transparent material serves to strengthen and to impart a high luster to the warp strands, thus enabling the use of cheap or weak materials for the layer 12 of backing material. For example, the layer 12 of backing material may comprise a sheet material having very little tensile strength, such as a short fibre paper or thin metal foil, in spite of which the finished fabric made in accordance with the invention has the appearance of an expensive material of high luster and interesting decorative color effects.

The article of the invention is especially adapted for use as a decorative material in wearing apparel and in all kinds of millinery material; also as wall hangings, curtains, draperies, lamp shades; ribbons and tying cords.

Since certain modifications in the article which embodies the invention may be made without departing from its scope, it is intended that all matter contained in the above description shall be interpreted as illustrative and not in a limiting sense.

It is also to be understood that the following claims are intended to cover all of the generic and specific features of the invention herein described, and all statements of the scope of the invention which, as a matter of language, might be said to fall therebetween.

I claim:

1. As an article of manufacture, a non-reversible woven fabric comprising series of warp and woof elements, the elements of one series comprising strips of a laminated material comprising at least two layers of sheet material held together by a layer of colored opaque adhesive, at least one of said layers of sheet material being transparent and at least one of said layers of sheet material being opaque, having a highly reflective surface.

2. As an article of manufacture, a non-reversible woven fabric comprising flat strands formed of strips of a laminated material comprising a flexible sheet of transparent material, a layer of colored opaque adhesive and a flexible sheet of opaque material, having a highly reflective surface, the optical appearance of one side of the fabric being imparted by the opaque sheet and the optical appearance of the other side of the fabric being imparted by the colored adhesive. 10

3. As an article of manufacture, a non-reversible woven fabric comprising strands formed of strips of a laminated material comprising a flexible sheet of transparent material, a layer of colored opaque adhesive and a flexible sheet of opaque material having a highly reflective surface. 15

4. As an article of manufacture, a non-reversible woven fabric comprising strands formed of strips of a laminated material comprising a flexible sheet of transparent material, a layer of opaque adhesive colored with a dyestuff and a flexible sheet of opaque material having a highly reflective surface. 20

5. As an article of manufacture, a non-reversible woven fabric comprising strands formed of strips of a laminated material comprising a flexible sheet of transparent material, a layer of opaque adhesive colored with an opaque pigment 30 and a flexible sheet of opaque material having a highly reflective surface.

6. As an article of manufacture, a non-reversible woven fabric comprising strands formed of strips of a laminated material comprising a flexible sheet of transparent, non-fibrous material, a layer of colored opaque adhesive and a flexible sheet of opaque material having a highly reflective surface. 35

7. As an article of manufacture, a non-reversible woven fabric comprising strands formed of strips of a laminated material comprising a flexible sheet of transparent regenerated cellulose, a layer of colored opaque adhesive and a flexible sheet of opaque material having a highly reflective surface. 40

8. As an article of manufacture, a non-reversible woven fabric comprising strands formed of strips of a laminated material comprising a flexible sheet of transparent material, a layer of colored opaque adhesive and a flexible sheet of material having a metallic surface. 45

9. As an article of manufacture, a non-reversible woven fabric comprising strands formed of strips of a laminated material comprising a flexible sheet of transparent material, a layer of colored opaque adhesive and a layer of metal foil. 50

10. As an article of manufacture, a non-reversible woven fabric comprising strands formed of strips of a laminated material comprising a flexible sheet of transparent regenerated cellulose, a layer of a colored opaque adhesive and a layer of metal foil. 60

11. As an article of manufacture, a fabric comprising a plurality of flat warp strands formed of strips of a laminated material comprising a flexible sheet of transparent material, a layer of colored opaque adhesive and a flexible sheet of opaque material having a highly reflective surface, and weft threads comprising a textile fibre. 65

JOSEPH W. STARK.